

1

2,997,365

PRODUCTION OF REGENERATED  
CELLULOSE FILAMENTS

John Oliver Smith, Coventry, and David Nicholson Tyler, Codsall, near Wolverhampton, England, assignors to Courtaulds Limited, London, England, a British company

No Drawing. Filed July 30, 1959, Ser. No. 830,477  
Claims priority, application Great Britain Aug. 12, 1958  
6 Claims. (Cl. 18—54)

This invention relates to the production of regenerated cellulose filaments from viscose and in particular to a process for the production of filaments having a high ratio of wet to dry tenacity, low extensibility, no skin-core differentiation and low water-imbibition.

We have found that by modifying or eliminating certain features of the basic viscose rayon process, highly oriented viscose rayon textile filaments having low extensibility can be produced.

The present process differs from the basic viscose rayon process in the following respects

(1) The use of a cellulose having a higher degree of polymerisation (D.P.). In practice this may lead to the elimination or shortening of mercerising or the ageing of the alkali cellulose.

(2) The use of a higher viscosity viscose. This is, to an extent, associated with the use of high D.P. cellulose, for only low cellulose concentrations of about 3 percent in the viscose could be used if normal ball-fall viscosities of, say, about 40 were to be used. However the increased viscosity assists in the rapid coagulation of the viscose during spinning and this is advantageous. The maximum increase in the viscosity is determined practically by the ability of the spinning equipment to handle the viscose. Thus a cellulose concentration of from 4 percent to 6 percent in the viscose and a viscose ball fall viscosity of over 50 and preferably from 100 to 200 may be used in practice.

(3) The use of a lower caustic soda concentration in the viscose which enables a low acid coagulation bath to be used. Such a bath can co-operate in the rapid coagulation of the filaments, but only slowly regenerates the cellulose. In practice the cellulose xanthate crumbs may be mixed with water rather than with the caustic soda solutions of normal viscose manufacture.

(4) The spinning of viscoses having higher salt figures so that an unusually large concentration of cellulose xanthate is present in the freshly extruded filaments and is preserved to a large extent in the filaments during the stretching operation, the more plastic cellulose xanthate molecules allowing more applied stretch than the relatively rigid regenerated cellulose molecules.

(5) The use of a coagulating bath containing much less acid, a lower sodium sulphate concentration and no zinc sulphate or only such zinc sulphate as is inevitably present as an impurity and in any case not more than 0.02 percent. The temperature of the bath should be between 20° C. and 30° C., that is to say lower than usual. All of these modifications are calculated to reduce the rate of regeneration of the cellulose.

(6) The use of a greatly reduced immersion path of the filaments in the bath, only sufficient to cause the filaments to coagulate so that they may be drawn from the bath without damage whilst preserving, as much as possible, the original xanthate groups of the viscose. The filaments are then in the very plastic condition required for the stretch which is applied outside the bath.

2

The necessary length of the immersion path varies with the denier of the filaments being spun.

(7) The stretch of at least 80 percent is applied to the filaments immediately they emerge from the bath. The plastic condition of the filaments makes the application of such a large stretch relatively easy and the filaments are fully regenerated only after the stretch has been applied.

The invention accordingly consists in a process for the production of viscose rayon filaments comprising extruding viscose having a cellulose content between 4 and 6 percent and a caustic soda content approximately half that of the cellulose, the cellulose having an average degree of polymerisation of at least 300 and the viscose having a salt figure of at least 10 and a ball fall viscosity of at least 50, preferably between 100 and 200, into a coagulating bath containing from 2.0 percent to 3.5 percent of sulphuric acid, less than 15 percent and preferably between 1 percent and 10 percent sodium sulphate, and not more than 0.02 percent of zinc sulphate as an impurity, maintaining the bath temperature between 20° C. and 30° C., limiting the length of the immersion path so that the filaments may be stretched by at least 80 percent of their original length on emerging from the bath, stretching the filaments immediately after they have emerged from the bath by at least 80 percent and subsequently completing the regeneration of the filaments.

The required immersion path of the filaments in the bath varies with the denier of the filaments. Thus for filaments having deniers up to 4.5 the immersion path should not exceed 6 inches and it is preferred for filaments having deniers of 3 or less that the immersion path should not exceed 3 inches.

The filaments can then be washed, dried and collected in a continuous form, or cut to produce a staple fibre, and subsequently washed and dried. Regeneration can be accelerated by treating the fibres at a suitable stage with warm dilute acid for example 2 percent of sulphuric acid at a temperature of 60° C.

The amount of sulphuric acid in the regenerating bath is kept within the stated range of 2.0 to 3.5 percent and it is preferably just sufficient to secure adequate coagulation. The actual amount varies with the number of filaments, the filament denier, spinning speed and the sodium sulphate concentration in the bath.

The highly oriented filaments of low extensibility can be made into fabrics having good dimensional stability and this is mainly due to the low imbibition of the filaments and their high initial wet modulus, that is the marked resistance of the wet fibres to stretch under low loads. The fabrics show reduced relaxation shrinkages and greatly reduced or eliminated progressive shrinkages.

These properties of the fabrics are similar to or better than cotton cloths of the same construction and are markedly superior to similar fabrics made from commercially available viscose rayon filaments.

The invention is illustrated by the following examples in which percentages are by weight.

60

*Example 1*

A high quality wood pulp such as that sold under the trade name Cordenier J. was steeped in an 18.6 percent aqueous solution of caustic soda for 1½ hours at 19° C. The surplus solution was removed by squeezing the pulp to a press ratio of 2.8 and the pulp was then disintegrated into crumbs for 2½ hours at 19° C. after which the

crumbs were allowed to age for 17 hours at the same temperature. The alkali cellulose was then xanthated for 3 hours with 42 percent of carbon disulphide (calculated on the original alpha-cellulose content of the wood pulp) at 24° C. and the resulting xanthate was mixed in a water-cooled vessel at 15° C. The mixing time was 3 hours during which the temperature rose to 17° C. A further 10 percent of carbon disulphide (also based on the alpha-cellulose) was then added in the mixer and the viscose was then filtered, deaerated by a flash deaeration process and left to age for 12 hours in vacuum.

The viscose, containing 5 percent of cellulose, 2.4 percent of caustic soda and 2.1 percent of sulphur and at a salt figure of 15, was then extruded at a ball fall viscosity of 100 seconds at 18° C. into a regenerating bath containing 2.7 percent of sulphuric acid and 1 percent of sodium sulphate at a temperature of 20° C. The viscose was extruded vertically upwards into the bath through a jet the face of which was about 1½ inches below the surface.

The filament bundle travelled vertically upwards through the bath and then a distance of 10 inches through the air onto two skewed sets of concentric discs of diameters 5, 6, 7, 8 and 9 inches respectively, giving 80 percent stretch for four stages. From the last disc the bundle was taken up on a roller and was stretched a further 17 percent between the last disc and the roller. It was then passed through a hot fixing bath containing 2 percent of sulphuric acid at a temperature of 90° C. in which it was stretched a further 3 percent. After washing and drying, the filaments had the following properties:

|                           |                      |
|---------------------------|----------------------|
| Filament denier           | 1.5                  |
| Conditioned tenacity      | grams per denier 3.6 |
| Wet tenacity              | do 2.6               |
| Extensibility conditioned | percent 6.0          |
| Extensibility wet         | do 8.0               |
| Water imbibition          | do 65.0              |

The cross-section of the filaments was circular and no differentiation between skin and core could be detected upon staining.

#### Example 2

Viscose prepared as in Example 1 was spun through 3 mil diameter holes into a bath containing 2.5 percent of sulphuric acid and 5.3 percent of sodium sulphate at a temperature of 23° C., the immersion being two inches. The thread was stretched a total of 100 percent in two stages and was then fully regenerated, washed, dried and collected. The final spinning speed was 50 metres per minute. The filaments produced had the following properties:

|                           |                       |
|---------------------------|-----------------------|
| Denier                    | 1.84                  |
| Conditioned tenacity      | grams per denier 3.62 |
| Wet tenacity              | do 2.46               |
| Extensibility conditioned | percent 8.3           |
| Extensibility wet         | do 10.6               |
| Water imbibition          | do 75.0               |

The cross-section was circular and showed no skin-core differentiation on staining.

#### Example 3

Viscose prepared as in Example 1, except that the crumbs were aged for 8 hours after disintegration, had a ball fall viscosity of 218 seconds at 15° C. The viscose was spun at a salt figure of 13 through a jet of 10,000 holes each of 2½ mille diameter at an extrusion ratio of 0.6 with two inches vertical immersion, into a bath containing 3.1 percent  $H_2SO_4$ , no zinc sulphate and 6.0 percent  $Na_2SO_4$ , at 22° C. The filaments were stretched by 95 percent of their original length, the final

spinning speed being 32 m./minute. The filament denier was 1.5 and the average properties of randomly chosen filaments were:

|   |                           |                       |
|---|---------------------------|-----------------------|
| 5 | Conditioned tenacity      | grams per denier 4.31 |
|   | Conditioned extensibility | percent 8.0           |
|   | Wet tenacity              | grams per denier 3.05 |
|   | Wet extensibility         | percent 10.4          |
|   | Water imbibition          | do 74.0               |

10

#### Example 4

Viscose as in Example 1 was spun at a salt figure of 12 through a jet having 10,000 holes each of 2½ mille diameter, with 2 inches vertical immersion into a bath containing 2.8 percent sulphuric acid, no zinc sulphate, and 9.0 percent  $Na_2SO_4$ , at 20° C. and the filaments were stretched by 100 percent of their original length outside the bath. The final spinning speed was 20 metres/minute and the denier 1.5. The filaments were cut to a staple length of 17½ inches, washed and dried. The average properties of the fibres were:

|    |                           |              |
|----|---------------------------|--------------|
| 25 | Conditioned tenacity      | 2.90         |
|    | Conditioned extensibility | percent 12.5 |
|    | Wet tenacity              | 1.80         |
|    | Wet extensibility         | percent 14.8 |

The staple fibres were spun into a yarn of 1/18's cotton count which was woven into a cloth of construction 64 ends/54 picks. 10 pounds of this cloth was 30 washed in soap at 60° C. in a rotary washing machine for 30 minutes, rinsed for 5 minutes at 40° C., rinsed again for 10 minutes at 40° C., hydroextracted and dried in a tumbler drier. The laundering cycle was repeated a number of times and the dimensions of the cloth measured at intervals. The results are shown in the following table.

| 40 | Wash                     | Percent shrinkage |      | Water imbibition (percent on weight of fabric) |
|----|--------------------------|-------------------|------|------------------------------------------------|
|    |                          | Warp              | Weft |                                                |
| 1  | loose dried<br>ironed    | 1.4               | 4.0  | 66                                             |
| 10 | loose dried<br>ironed    | +1.2              | 1.4  | -----                                          |
| 45 | 25 loose dried<br>ironed | 4.2               | 4.8  | -----                                          |
|    |                          | 0.6               | 1.0  | -----                                          |
|    |                          | 4.6               | 5.0  | -----                                          |
|    |                          | 1.0               | 1.8  | 60                                             |

It will be noted that the properties of the fabric are equivalent to or better than cotton in a cloth of the 50 same construction and are much improved compared with normal viscose rayon textile fibres in a cloth of the same construction.

What we claim is:

1. A process for the production of viscose rayon filaments comprising extruding viscose having a cellulose content between 4 and 6 percent and a caustic soda content approximately half that of the cellulose, the cellulose having an average degree of polymerization of at least 300 and the viscose having a salt figure of at least 60 10 and a ball fall viscosity between about 50 and about 200 seconds at 18° C., into a coagulating bath containing from 2.0 percent to 3.5 percent of sulphuric acid, less than 15 percent sodium sulphate, and not more than 0.02 percent of zinc sulphate as an impurity, to form filaments, maintaining the bath temperature between 20° C. and 30° C., removing the filaments from the bath while they are still capable of being stretched in air at least 80% of their original length, stretching the filaments in air immediately after they have been removed 65 from the bath by at least 80% and completing the regeneration of the filaments after they have been stretched.
2. A process for the production of viscose rayon filaments having deniers of up to 4.5 according to claim 1, in which the length of the immersion path of the filaments in the bath is not more than 6 inches.

3. A process for the production of viscose rayon filaments having deniers of up to 3 according to claim 1, in which the maximum length of the immersion path of the filaments in the bath is 3 inches.

4. A process as claimed in claim 1 in which the bath contains from 1 percent to 10 percent of sodium sulphate.

5. A process as claimed in claim 1 in which the ball fall viscosity of the viscose is between 100 and 200.

6. A process as claimed in claim 1 in which the salt figure of the viscose is at least 12.

References Cited in the file of this patent

UNITED STATES PATENTS

|           |           |                |
|-----------|-----------|----------------|
| 2,611,928 | Merion    | Sept. 30, 1952 |
| 2,732,279 | Tachikawa | Jan. 24, 1956  |
| 2,775,505 | Pedlow    | Dec. 25, 1956  |